

## UNITED STATES PATENT OFFICE

2,279,565

## FLUX

James Fletcher, Detroit, Mich., assignor of one-half to Frank Kuhn, as trustee for Airielle C. Kuhn, both of Detroit, Mich.

No Drawing. Application April 21, 1941,  
Serial No. 389,606

5 Claims. (Cl. 75—65)

The present invention relates to fluxes for use in connection with metallurgical processes and particularly in the melting and casting of metals and alloys.

In the melting and casting of non-ferrous metals and alloys, especially those consisting chiefly of copper with other elements such as chromium or silicon, or both, the use of the usual fluxes does not result in sufficient fluidity of the melt to permit easy flow.

Among the objects of the present invention, therefore, is a flux, the use of which permits the obtaining of a melt which flows readily and which seems in itself to aid in the reduction of the metal to thin fluidity.

The flux which forms the subject matter of the invention and which will effect the above results is a mixture of borax, preferably calcined or anhydrous, and lime, preferably finely powdered air-slaked lime. These two materials are preferably mixed before use and used in proportions which may vary from about 1 to 1 to about 1 to 2 of borax and lime respectively, these proportions may be either by volume or by weight since their specific gravity does not greatly differ and since, for the purpose, the proportions are not critical.

In the use of the mixture, the borax first melts and then reacts with the lime with evolution of gases, probably  $\text{CO}_2$  and water vapor, to produce a quite fluid cover liquid.

While the exact effect of the flux upon the metals is not known, it is believed that it exerts a de-oxidizing effect since easily oxidizable metals

like copper and aluminum melt and become quite fluid when this flux is used, while the same metals at the same temperatures merely become soft and too viscous to flow, when ordinary fluxes are used.

Further, while the metals mentioned hereinbefore are all non-ferrous, the flux may also be used with advantage in the melting of the ferrous alloys.

10 I claim:

1. A flux for use in the melting of non-ferrous metals consisting of a mixture of anhydrous borax and air-slaked lime in the proportions ranging from substantially 1:1 to 1:2 of the two substances respectively.

2. A flux for use in the melting of non-ferrous metals consisting of a mixture of anhydrous borax and lime in substantially equal proportions.

3. The process of fusing non-ferrous alloys 20 consisting largely of copper which comprises melting such alloys in the presence of a mixture of borax and lime.

4. The process of fusing non-ferrous alloys 25 consisting largely of copper which comprises melting such alloys in the presence of a mixture of anhydrous borax and airslaked lime.

5. The process of fusing non-ferrous alloys 30 consisting largely of copper which comprises melting such alloys in the presence of a mixture of borax and lime in substantially equal proportions.

JAMES FLETCHER.